

CATION OF TEXTILES &amp; F

1,927,839

9/26/1933

## UNITED STATES PATENT OFFICE

1,927,839

CLEANING MEDIUM FOR ANIMAL AND  
VEGETABLE TEXTILE FIBERS OR TEXTILE MATERIALS

Carl Lüdecke and Wilhelm Wilcken, Berlin, Germany

No Drawing. Application August 11, 1930, Serial  
No. 474,655, and in Germany January 7, 1929

1 Claim. (CL. 87-5)

The present invention relates to a method of cleaning animal and vegetable textile fibers or textile materials.

For the purpose of general preparation and for the removal of the mechanically adhering impurities and also the oil, fat, wax, resin or bitumen present in the natural state or added during the treatment, the vegetable or animal fibers required for the production of textile materials,

or also the yarns, fabrics, etc. made from the same, are—mostly after a preliminary washing, digestion or roasting operation—treated with weak alkaline solutions or alkaline soap solutions at increased temperature. It has also been

proposed to employ alkaline soaps with the addition of a small quantity of solvent for the same purpose.

Whereas, generally speaking, alkalis are deleterious to textile fibers as they act to reduce the breaking strength of the fibers, and make the same brittle and difficult to spin, there is more particularly in the case of animal fibers, for example raw wool, an additional weakening of the material by reason of the fact that the same is

robbed by the alkali of the natural sulphur content, thus being deprived of its reducing property. Both raw wool as well as wool products or partly finished products are extremely sensitive to relatively high temperatures. The hy-

drolyzation products, which are particularly important as regards the feel, the strength and the finish of the wool are expelled by the heat, this also applying to the keratins, albumins, globulins, collagens and other albumen substances

contained in animal and vegetable fibers and causing their elasticity. An additional disadvantage associated with the hitherto-known methods of cleaning raw fibers consists in the fact that any assaulting fatty substances emulsify during the cleaning operation by reason of saponification resulting from the alkalis and alkaline soaps employed, and can only be removed again with a considerable amount of trouble, whereby impurification by reason of the fatty acids contained in the soap and likewise separated during this operation is not to be avoided.

The textile fibers, yarns, fabrics, etc. freed from all impurities and thoroughly washed may be subjected to the additional bleaching or other processes by treatment with bleaching agents

acting in a reducing or oxidizing manner, or to any other desired treatment. The performance of the complete operation, which in reality consists of a number of consecutive digesting and

cleaning processes, necessitates large and expensive apparatus and a considerable amount of space.

According now to the present invention the fibrous material is accorded very extensive consideration and a much higher class product obtained by reason of the fact that both the use of alkalis or alkaline soaps as well as the application of increased temperatures is dispensed with, an acid preparing and cleaning agent, preferably in cold solution, being employed in place thereof. For removing the fatty impurities fat-dissolving agents of different kinds, or mixtures of these, are employed, converted into an emulsion by the use of a thickening vegetable mucus as protective colloid and stabilizer in acid dispersion, which emulsion may, if desired, be mixed with water.

The agent causing the dissolution of the oleous, fatty, waxy, resinous and bituminous substances consists of a mixture of volatile, organic fat-dissolving substances, the total density of which is approximately equal to that of the viscous dispersion agent.

The bleaching action on the raw or also pre-treated or partly worked fibers is produced by the use of a weak acid or an acid salt solution or any suitable compound or mixture, which is readily capable of being expelled by rinsing, and which induces the textile fibers to be opened out and thus give off the impurities they contain without disturbing the colloidal aggregation. We have discovered that, inter alia, the following substances are particularly suitable for the stated purpose: sulphurous acid, sodium bisulphite, hydrosulphite, chloro-sulphonic acid, boric acid, phosphoric acid, benzoic acid, formic acid, oxalic acid, tartaric acid, lactic acid or compounds thereof, if necessary with the addition of peroxides or other agents acting in an oxidizing or reducing sense. The nature and the quantity of the acid addition depends on the nature of the fiber and on the desired bleaching action.

According to the invention there is employed as emulsion negotiating medium between the fat solvent phase and the acid watery dispersion agent for forming the necessary colloidal fat solvent-in-water emulsion a proteinous vegetable mucus in a certain proportion suitable for producing a sol condition, and this may be gum, alga or also moss and tang mucusses, viz., mixed with each other or with one of the vegetable mucusses in a concentration producing a colloidal state. The homogeneous dispersion of the ingredients causing the cleansing of the fibers, which is thus obtainable, may, according to the invention, be

additionally stabilized by adding to the emulsion a certain quantity of alcoholic formalin solution until by reason of the same the stickiness and the water-solubility of the mucusses contained in the emulsion are in part again eliminated without 5 affecting the gelatinous soak. In certain instances a satisfactory cleansing action in cold solution may be obtained by the liquid fat-dis-  
solving agents and the proteinous vegetable 10 mucusses alone, which are included in the clean-  
ing agent, as the mucusses pick up and mechani-  
cally bind the fatty and other impurities sepa-  
rated from the fibers, and thus become charged 15 with the same, so that these may be readily ex-  
pelled upon the rinsing operation. It has further-  
more been ascertained that this effect may be still 20 further amplified by a small addition of sour milk  
or skimmed milk, the cleaning and bleaching ef-  
fect of which may be assumed to be readily known,  
the milk proteins in conjunction with the pro-  
teins of the vegetable mucus improving the emul- 25 sion system.

This emulsion, containing more or less acid, 30 may be mixed with water in any desired propor-  
tion, and may accordingly be readily converted  
into the diluted form necessary for use.

The solubility in respect of the fatty substance 35 of the fibers is, by reason of the extremely inti-  
mate dispersion, which is obtained by the me-  
chanical homogeneousness, of the atomized par-  
ticles of solvent surrounded by a protective col-  
loidal coating in the soaked viscous mucous solu- 40 tion, greater than when using the solvent alone.

A fine emulsion of this kind with colloidal dis-  
persion is capable of penetrating deeply into the 45 moist fibers and of there exerting a vigorous  
action in the dissolution of the fatty substances  
which may be present. The same accordingly  
fulfils the purpose of the alkaline soap lyes other-  
wise usually employed, but in more complete fash- 50 ion and also in a manner which does not have the  
same detrimental action on the fibers. The sol-  
vent charged with the fatty substances and the  
like may be readily expelled from the fibers with-  
out trace by the use of cold rinsing water.

The mucous colloidal dispersion agent not only 55 exerts a fixing action of the emulsified solvent  
on the fatty textile fibers, but also prevents too  
sudden action of the acid on the substance of  
the fibers. Due to the protein content of the  
vegetable mucus, the fibers are maintained in a 60 pliable condition, as these fibers absorb said  
mucus after the fat has been removed. In this  
manner not only is the exposed fiber strength-  
ened in its structure, but also the power of ab-  
sorption and accordingly its dyeing capability 65 and adaptability for spinning purposes are in-  
creased without losing in any way extensibility  
and weight, so that the fibers or fabric has a  
softer touch and a smoother and more glossy  
appearance.

65 The mucous colloidal dispersion agent is also  
capable of greatly reducing the risk of water  
absorption and loss of volume in the fibers  
when the fibers are dried, as the water is  
absorbed by the mucous substance and not by the  
70 fiber itself. The addition of a small amount of  
water to the emulsion will not affect the  
cleaning and bleaching action, but will  
adversely affect the water absorption and  
the water absorption will be reduced, great proportion- 75

An additional advantage associated with the  
use of the cleaning agent according to the in-  
vention consists in the combination thus ren-  
dered possible of the single preparing, cleaning  
and bleaching operations in one single process,  
the complicated cleaning operation distributed  
over a plurality of baths hitherto usual thus be- 80 ing unnecessary.

Apart from those fibers which may be placed  
under the general heading of textile fibers, and  
consisting for example of wool, silk, seed, bast,  
fruit, leaf, straw, wood and other cellulose fibers,  
it is also possible to clean with the method ac-  
cording to the invention other products or ma- 85 terials such as feathers, hair, furs, etc.

90 Examples of the solvent employed are quoted  
in the following:

Example 1.—40 parts of a 6% tragacanth so-  
lution are mixed with 15 parts of a 10% car-  
ragheen or Irish moss mucous solution and 10  
parts of a 3% agar-agar solution and stirred 95  
with 25 parts of a mixture composed of heavy  
benzine and trichlorethylene, the specific weight  
of which at 15° is little more than 1, for instance,  
a mixture composed of 60% heavy benzine hav-  
ing 0.780/35 specific weight and 40% trichlor-  
ethylene. After the addition of a solution of 2  
parts oxalic acid and 1 part sodium bisulphite  
in 6 parts of water vigorous stirring is performed,  
and when a homogeneous emulsion has been ob- 100  
tained one part of a mixture is added comprising  
formalin and butylalcohol in equal parts.

Example 2.—A further emulsion having a con-  
siderable solvent addition is produced by mixing  
35 parts of a 9% tragacanth solution with a so-  
lution comprising 1 part tartaric acid and 5 parts  
of sour milk in 14 parts of water and stirring in  
45 parts of a solvent mixture composed of equal  
parts of heavy benzine and trichlorethylene.

110 It will be understood that no restriction is  
made to the specific details described or to the  
examples above quoted, but that various modifi-  
cations are quite possible within the meaning of  
the annexed claim without departing from the  
spirit of the invention.

115 What we claim as new and desire to secure by  
Letters Patent is:

A cleaning and purifying medium for animal  
and vegetable textile fibers and substances, con-  
sisting of an emulsion mixable with water and  
comprising an aqueous solution of an acid used  
as the dispersion medium, a volatile water-im-  
miscible organic fat solvent used as the dispersed  
substance, a vegetable mucous substance acting  
as a thickening medium and used as the stabilizer  
of the emulsion, and sour milk.

CARL LÜDECKE,

WILHELM WILCKEN.

135

140 The invention is not limited to the specific  
examples given, but may be modified in many  
ways without departing from the spirit of the  
invention. For example, the acid may be  
any acid which is capable of decomposing  
the fat, and the fat may be any volatile  
145 organic fat which is capable of being  
dispersed in an aqueous solution. The  
mucous substance may be any mucous  
substance which is capable of stabilizing  
the emulsion and of being dispersed in  
150 an aqueous solution. The solvent may  
be any volatile organic solvent which is  
capable of dispersing the fat in an  
aqueous solution.